

July 22, 1952

C. STERN

2,604,418

TIMEPIECE DIAL

Filed Feb. 17, 1948

FIG. 1



FIG. 2



FIG. 3



FIG. 4



FIG. 5



Inventor  
Charles Stern  
By Robert E. Burns  
Attorney

## UNITED STATES PATENT OFFICE

2,604,418

## TIMEPIECE DIAL

Charles Stern, Geneva, Switzerland

Application February 17, 1948, Serial No. 8,839  
In Switzerland February 18, 1947

1 Claim. (Cl. 148—6.1)

1

The present invention relates to time-piece dials and has particular reference to a process of manufacturing time-piece dials having prominent indicia members stamped therefrom.

It is an object of the invention to provide time-piece dials of base metal or alloys having prominent indicia members stamped therefrom and durably colored in a color different from that of the dial plate itself.

According to an important feature of the invention prominent indicia members are stamped from a plate of light metal or alloy such, for example, as aluminum or magnesium or their alloys, and the whole plate is subjected to an oxidizing treatment, preferably to anodic oxidation; the plate is then covered by a layer of commonly known masking material, leaving the prominent indicia members uncovered, then immersed in a dye bath and the masking material removed after dyeing, whereby the prominent indicia members are durably colored in a color different from that of the plate from which they are stamped.

The accompanying drawing illustrates the various steps of the invention.

Fig. 1 is a plan view of a watch dial embodying the invention;

The Figures 2 to 5 are enlarged sectional views taken on line A—A of Fig. 1 showing a portion of the dial after various steps of the manufacturing process.

In carrying out the process, I stamp prominent indicia members, for instance hour characters as 2, from a plate 1 made of light metal or alloy such as aluminum, magnesium, aluminum alloy or magnesium alloy; I then submit the plate to an oxidizing treatment, either chemically or electro-chemically, preferably to anodic oxidation, whereby the whole upper surface of the plate including the faces of the prominent indicia members is provided with a layer 3 of aluminum or magnesium oxide, as shown in Fig. 3. The next step is to cover or save the upper surface of the plate by a layer 4 of masking material such as cellulosic varnish which leaves uncovered the surfaces 5 of the indicia members 2.

The next step is to dye the oxidized surfaces 5 of the indicia members, as by immersion of the dial in a hot dye bath, and then to remove the masking material 4 as by immersion of the dial in a suitable solvent.

A dial is thus obtained having prominent hour characters or other indicia members, the upper surface of which is durably colored, for instance in blue, red or yellow, and thus more neatly

2

stands out in relief on the background of the dial which may be for example white, shining or of dull satin finish.

Optionally, after oxidation and masking of the plate, the prominent indicia members may be uncovered and polished by means of abrasive material, then oxidized and dyed.

Optionally also, the prominent indicia members may be polished and masked before the oxidizing treatment and the background of the dial

10 given a satin finish by well known process; then, after removal of the masking material from the indicia members, the whole may be oxidized, the background masked and the indicia members dyed as hereinbefore described.

What I claim is:

A process for manufacturing time-piece dials comprising the steps of stamping prominent indicia members from a plate of light metal of the 20 group consisting of aluminum, magnesium and alloys of said metals polishing the prominent indicia members and covering them with masking material, giving the background of the plate a satin finish, removing the masking material from 25 the indicia members, oxidizing the whole plate together with the prominent indicia members, protecting the background of the plate by covering it by a layer of masking material leaving the prominent indicia members uncovered, dyeing the uncovered indicia members and removing 30 the masking material from the background.

CHARLES STERN.

## 35 REFERENCES CITED

The following references are of record in the file of this patent:

## UNITED STATES PATENTS

| 40 | Number    | Name      | Date          |
|----|-----------|-----------|---------------|
|    | 430,424   | Eaton     | June 17, 1890 |
|    | 864,467   | Ingraham  | Aug. 27, 1907 |
|    | 1,304,749 | Divine    | May 27, 1919  |
| 45 | 1,821,561 | McFarland | Sept. 1, 1931 |
|    | 2,516,986 | Heinse    | Aug. 1, 1950  |

## FOREIGN PATENTS

| 50 | Number  | Country       | Date          |
|----|---------|---------------|---------------|
|    | 445,242 | Great Britain | Apr. 6, 1936  |
|    | 483,776 | Great Britain | Apr. 26, 1938 |
|    | 65,167  | Switzerland   | Mar. 4, 1913  |

## OTHER REFERENCES

V. F. Henley, The Metal Industry (London),  
55 June 18, 1943, page 388.